

United States Patent [19]  
Foreman

[11] 3,793,208  
[45] Feb. 19, 1974

[54] **METHOD OF RECTIFYING COMMERCIAL SALT BATHS**

[75] Inventor: **Robert W. Foreman**, Bloomfield Hills, Mich.

[73] Assignee: **Park Chemical Company**, Detroit, Mich.

[22] Filed: **Jan. 4, 1973**

[21] Appl. No.: **320,885**

[52] U.S. Cl. .... **252/71**, 148/15, 148/22

[51] Int. Cl. .... **C09k 3/02**

[58] Field of Search... **252/71**; 148/15, 15.5, 22, 27, 148/28

[56] **References Cited**

UNITED STATES PATENTS

183,804 4/1876 Herrenschmidt ..... **252/71**

|           |         |                         |          |
|-----------|---------|-------------------------|----------|
| 2,205,180 | 6/1940  | Shaver .....            | 252/71 X |
| 2,278,297 | 3/1942  | Wood .....              | 252/71   |
| 2,375,758 | 5/1945  | Bates .....             | 252/71   |
| 2,375,759 | 5/1945  | Kalichevsky et al. .... | 252/71   |
| 2,375,760 | 5/1945  | Fahnestock .....        | 252/71   |
| 2,375,761 | 5/1945  | Bates .....             | 252/71   |
| 2,857,301 | 10/1958 | Mauzy et al. ....       | 252/71 X |
| 3,220,893 | 11/1965 | Blackwood et al. ....   | 148/28   |
| R23,017   | 7/1948  | Bates .....             | 252/71   |

Primary Examiner—Leon D. Rosdol

Assistant Examiner—Harris A. Pitlick

Attorney, Agent, or Firm—Harness, Dickey & Pierce

[57] **ABSTRACT**

A method of rectifying commercial salt baths which operate generally within the temperature range from about 300°-600° F, said rectifying being to remove undesirable carbonates and/or hydroxides impurities.

7 Claims, No Drawings

## METHOD OF RECTIFYING COMMERCIAL SALT BATHS

### BACKGROUND OF THE INVENTION

This invention broadly relates to a method of rectifying commercial salt baths. The state of the art is indicated by the following U. S. Pat. Nos.: 2,278,297; 2,375,758; 2,375,759; 2,375,760; 2,375,761; Re 23,017; and 2,474,680.

Accordingly, it is a primary object of this invention to provide a new improved method of rectifying commercial salt baths to remove undesirable carbonates and/or hydroxides impurities therefrom.

Other objects, features, and advantages of the present invention will become apparent from the subsequent description and the appended claims.

### SUMMARY OF THE INVENTION

Briefly stated, the present invention concerns a method of rectifying in situ a commercial salt bath containing undesirable carbonates and/or hydroxides impurities, comprising the steps of: maintaining the bath at a temperature from about 300°F to about 600°F; introducing into the bath, an aqueous solution consisting essentially of, about 0.1 percent to about 8 percent by weight free nitric acid, about 0.01 percent to about 5 percent by weight non-ionic surface active agent means for deterring foaming of the bath and for assisting in rapid dispersion of the solution in the bath, and the balance water, to thereby rectify the bath.

### DESCRIPTION OF PREFERRED EMBODIMENTS

The invention discovered and disclosed herein has been found to provide a surprisingly good and unexpectedly advantageous way of rectifying commercial salt baths for the purpose of removing or converting undesirable carbonates and/or hydroxides impurities in these commercial salt baths, such that these impurities are no longer present in the bath or are present in such low amounts that they do not harmfully affect the operation of the bath.

Nitrate-nitrite salt baths accumulate alkali and alkali carbonate impurities in use due either to thermal decomposition or drag-in from carbonate containing higher temperature baths. The alkali (sodium hydroxide or potassium hydroxide) or alkali carbonate (sodium carbonate or potassium carbonate) impurities are undesirable for efficient salt bath heating and quenching of steel.

The discovery has been made in this invention that it is possible to eliminate difficult separation and removal of the carbonates or alkalis from molten nitrate/nitrite salt baths which operate at a temperature of about 300°-600°F. These carbonates or impurities are sparingly soluble in such baths at their usual operating temperatures (300°-600°F) and they interfere with both heat transfer and quenching efficiency.

In the past it has not been known that such salt baths could be rectified in situ, that is, in accordance with this invention it is not required to take the liquid bath material through any kind of an external treating system or the like. Furthermore it has been discovered in this invention that the concentration of the nitric acid used and referred to above is critical in successfully carrying out the invention herein. Still further in this invention the discovery has been made that unique re-

sults appear to be obtained through the use of a surface active agent means which are discussed and disclosed herein. The temperature at which the salt bath is maintained is also important. Below about 400°F, heavy brown fumes are liberated if it is attempted to carry out the method herein and particularly if it is attempted to carry out the method herein below 300°F then the heavy brown fumes liberated become very excessive. Preferably, the method herein should be carried out at a temperature range between about 400°F and 400°F.

The nitric acid content of the aqueous solution referred to above should preferably be maintained within the range of about 2 percent to about 7 percent and best results are obtained within the range of about 4 percent to about 6 percent free nitric acid by weight of said aqueous solution.

The surface active agent means used in the inventive method herein should be non-ionic, low-foaming, and soluble in water and stable to dilute aqueous acids such as nitric acid. The surface active agent means should preferably be composed of carbon, hydrogen and oxygen to avoid undesirable residues in the rectified salt bath (that is undesirable residues such as phosphates or sulfates). Desirable surface active agent means for the purpose of carrying out the inventive discovery herein are as follows:

|    | Trade Name          | Supplier                    | Physical-chemical Description                                                                                                            |
|----|---------------------|-----------------------------|------------------------------------------------------------------------------------------------------------------------------------------|
| 30 | Pluronic F68LF      | BASF/Wyandotte Chemical Co. | Condensate of ethylene oxide with hydrophobic bases formed by condensing propylene oxide with propylene glycol, 100% Active Flaked solid |
| 35 | Igepal CO 610       | GAF Corporation             | Nonylphenoxy poly (ethyleneoxy) ethanol, 100% active liquid low-foaming in water                                                         |
| 40 | Poly-Tergent LF-405 | Olin Corporation            | Polyethenoxy ether, 99% active liquid                                                                                                    |
| 45 | Triton CF-21        | Rohm & Haas Co.             | Alkyaryl polyether 100%, active liquid low-foaming in H <sub>2</sub> O                                                                   |
|    | Tergitol Min-Foam   | Union Carbide Corporation   | Modified linear alcohol ethoxylate. low foam, 100% active liquid surfactant                                                              |

50 The carbonates impurities referred to herein are normally salts of barium, sodium, potassium, or calcium and are normally present in the commercial salt bath from about 0.01 percent to about 3 percent by weight of the salt bath. The hydroxides impurities referred to herein are normally alkali hydroxides and may be present in the salt bath being rectified from about 0.01 percent to about 50 percent by weight.

55 In order to further illustrate the invention the following example is provided. It is to be understood however that the example is included for illustrative purposes and is not intended to be limiting of the scope of the invention as set forth in the subjoined claims.

### EXAMPLE

60 A composition is prepared consisting of 5 percent by weight free nitric acid, 0.1 percent by weight of a surface active agent means (F68LF) and the balance water to 100 percent by weight. A commercial salt bath

(of approximately 1,000 pound size) to be rectified was first analyzed to determine the percentage of sodium carbonate therein in percent by weight. The percent by weight of sodium carbonate was determined to be approximately  $\frac{1}{2}$  percent by weight sodium carbonate. 5 Approximately 14 gallons of the above rectifying composition is added to the commercial salt bath. The result is that the commercial salt bath is satisfactorily rectified by the addition of said 14 gallons of the rectifier composition above. It has been found that approximately 2.8 gallons of said above rectifier composition will normally rectify the undesirable carbonate impurity in a 1,000 pound nitrate commercial salt bath per each 1/10 percent by weight of sodium carbonate impurity in said bath. Additional amounts of said rectifying composition may be necessary to rectify the undissolved carbonates impurities lying at the bottom of the commercial salt bath which undissolved carbonates will not go into solution in the bath unless and until the already dissolved carbonates in the bath are rectified or 10 removed from the bath through addition of said rectifying composition.

While it will be apparent that the preferred embodiments of the invention disclosed are well calculated to fulfill the objects above stated it will be appreciated 25 that the invention is susceptible to modification, variation, and change without departing from the proper scope or fair meaning of the subjoined claims.

What is claimed is:

1. A method of rectifying in situ a metal heat treating 30 molten nitrate/nitrite salt bath containing undesirable carbonates and/or hydroxides impurities, comprising the steps of:

maintaining the bath at a temperature from about

300°F to about 600°F; introducing into the bath, an aqueous solution consisting essentially of, about 0.1 percent to about 8 percent by weight free nitric acid, about 0.01 percent to about 5 percent by weight non-ionic surface active agent for deterring foaming of the bath and for assisting in rapid dispersion of the solution in the bath, and the balance water, to thereby rectify the bath.

2. The method of claim 1 wherein, said nitric acid is present from about 2 percent to about 7 percent.

3. The method of claim 1 wherein, said nitric acid is present from about 4 percent to about 6 percent.

4. The method of claim 1 wherein, said temperature is from about 400° to about 600°F.

5. The method of claim 4 wherein, said nitric acid is present from about 4 percent to about 6 percent.

6. The method of claim 1 wherein, said surface active agent is selected from at least one of the group consisting of a polyethenoxy ether liquid and an alkyaryl polyether liquid.

7. The method of claim 1 wherein, said carbonates are salts of barium, sodium, potassium or calcium and are present in the bath from about 0.01 percent to about 3 percent by weight, and said hydroxides are present in the bath from about 0.01 percent to about 50 percent by weight.

\* \* \* \* \*

UNITED STATES PATENT OFFICE  
CERTIFICATE OF CORRECTION

Patent No. 3,793,208 Dated February 19, 1974

Inventor(s) Robert W. Foreman

It is certified that error appears in the above-identified patent and that said Letters Patent are hereby corrected as shown below:

Front page, column 2, References, last reference, "R23,017"  
should be --Re23,017--.

Column 2, line 10, second occurrence of "400° F" should be  
--600° F--.

Signed and sealed this 21st day of May 1974.

(SEAL)

Attest:

EDWARD N. FLETCHER, JR.  
Attesting Officer

C. MARSHALL DANN  
Commissioner of Patents